

## UNITED STATES PATENT OFFICE

2,185,081

## METHOD OF MAKING ALLOYS OF IRON AND STEEL

Casimir James Head, Montreal, Quebec, Canada, assignor to Metallurgical Development Company Limited, Montreal, Quebec, Canada, a corporation of Quebec, Canada.

No Drawing. Application March 25, 1939,  
Serial No. 264,212

10 Claims. (Cl. 75—133)

This invention relates to an improved method for alloying metals, particularly iron and steel, with other metals reducible from their oxides, and more especially for the production of steels having a high percentage of the alloying metal with a negligible or low percentage of carbon, and the present case is a continuation in part of my application for Letters Patent, Serial No. 147,736, filed under date of June 11, 1937, for a Method of making alloys of iron and steel, and which application was allowed under date of October 8, 1938.

Primarily the process of the present invention is for alloying a bath of ferruginous molten metal whereby an oxide of the alloying metal in combination with a suitable reducing agent, such as a metal silicide, both in a comparatively fine state of division, are bound together with a suitable hydroxide of an alkaline earth such as slaked lime, or with a chloride solution of an alkaline earth, such as chloride of magnesium, and just sufficient water is added to form a plastic mass, the amount of such binding material used being sufficient to bind these ingredients together, and to partly flux the silica formed by the chemical reactions as therein expressed; the quantity of the hydroxide or chloride of an alkaline earth needed to effect this, and to maintain the molded pieces or blocks of sufficient density for the purpose when introduced into the furnace chamber that they will penetrate the slag and come into direct contact with the surface of the bath of ferruginous molten metal, generally varies from 10 to 12 parts to 100 parts of the mix (ore and the metal silicide); the plastic mass is pugged up in any suitable mill and may be molded into comparatively heavy pieces or blocks weighing about 40 to 50 lbs. or more, and may be of any suitable shape and size and weight for the furnace men to handle. These molded pieces or blocks, after being air dried at room temperature, or the drying may be hastened by a current of air, may preferably be treated with a milk of lime wash, and after being sufficiently dried are transferred to a suitable oven or kiln where the excess or loosely held water is expelled. They are then further heated up to a comparatively high temperature in this chamber or transferred to a separate chamber for this purpose, the object being to drive off any contained water held by the pugged mass of alloying material and the alkaline earth together, and the air drying of the pieces, and also of any carbonic acid gas ( $CO_2$ ) that the lime may have

absorbed before being charged into the melting furnace chamber for alloying purposes.

While in the practical operation of my invention a temperature in excess of  $1650^{\circ}$  F. has proven satisfactory for freeing the pieces or blocks of alloying material from free and combined water therein and to degasify same, nevertheless it has been found that the temperature range for accomplishing this desirable result, as well as to entirely free the pieces or blocks from gases, is largely dependent upon the characteristics and nature of the alloying material and of the alkaline earth used, which are component parts of the molded pieces or blocks, and therefore the temperature may vary from  $700^{\circ}$  C. to  $1000^{\circ}$  C. The object of this final heating within said range of temperatures being to liberate any remaining free water as well as the combined and colloidal water held by the pieces or blocks, and any carbonic acid gas that they may have absorbed, so that when the heated pieces or blocks are charged into the furnace chamber, the bath of ferruginous molten metal will not absorb gases therefrom, and by virtue of their density, weight, and heat will displace the slag and come into direct contact with the surface of the molden bath of ferruginous metal, and as the reduced metal or metals are released from the pieces or blocks they will carry the heat evolved by the exothermic reaction and pass directly into the metal bath, under protection of the slag covering, and thus substantially prevent the reduced alloying metal or metals becoming oxidized and passing off into the slag.

In carrying forward the invention upon these lines it has been found that important features are that the process involving the use of the invention supplies a simple, cheap and efficient means for alloying a bath of ferruginous molten metal with the alloying metal, such as chromium, since the ore of the alloying metal may be applied direct to the molten body or bath of the metal to be alloyed; and, according to the present invention it is possible to use a lower grade of alloying ore (such as a low grade ore containing chromium) than was heretofore possible. It has actually been determined in practice that according to the present invention the alloying process can successfully be carried out with the use of a low grade chrome ore having a ratio of chromium to iron of 1.7 to 1, that is, an ore having approximately 40% chromium sesquioxide, whereas according to prior practices it has only been possible to successfully carry out the alloying operation with the use of a more

costly high grade chrome ore having a ratio of 3 to 3½ of chromium to 1 of iron, that is an ore averaging about 50% Cr<sub>2</sub>O<sub>3</sub>.

Also, an important consideration in carrying forward the invention is that it can be applied, without alterations, to existing plants which operate either the basic open hearth or basic electric furnaces and that at the termination of the alloying period, according to the present invention, the molten bath of metal is thoroughly deoxidized and maintains sufficient heat and fluidity for tapping and teeming.

Furthermore, in carrying out the method of alloying, according to the present invention, the resulting ingots are sound and satisfactorily forged out, and upon rolling into strip a pronounced feature of importance has been found in the fact that the edges of the strip are free from rupture and ragged selvage, such as ordinarily occurs and must be removed as scrap, with consequent loss. Ordinarily high chromium content steels are not made in the open-hearth furnace owing to the strong oxidizing atmosphere of this furnace, but under my procedure herein explained, it is possible to produce such steel in the open-hearth furnace and the direct loss by oxidation of the alloyed chromium would be considerably less, since my process uses a cheaper low grade chromium as against the more costly specially made low-carbon ferro-chrome.

It has also been found that finished material made according to the present invention presents a finer and denser grain and smoother surface than is known to the applicant in any finished alloyed material made according to any present or standard practice.

As distinguished from prior practices which are operated at relatively high cost, and with highly specialized technique, and in some cases under prohibitive and dangerous conditions, the present invention generally has in view an economical and efficient method of making iron or steel alloy having a high percentage of alloying metal with a low carbon content, which method can be carried out satisfactorily in either an open-hearth or an electric furnace; also the present invention involves the use of inexpensive alloying and reducing materials, the reactions between which are exothermic and utilized to keep the metal hot and fluid.

And finally, it is an object of the present invention to provide an improved method of making low carbon, high chromium or other alloy steels in which the alloying and reducing materials are maintained in contact with the surface of the metal bath below the slag during reduction, so as to accelerate the reduction and prevent the alloying metal from becoming oxidized and passing into the slag.

These and other objects are attained by the improvements comprising the present invention, which may be stated in general terms as comprising a method of making an alloy iron or steel and/or other alloyable metals, including the step of adding to the metal bath relatively heavy molded blocks containing one or more oxides of the alloying metal and a metal silicide, said blocks being adapted to penetrate the slag and come in direct contact with the surface of the molten metal of the bath.

By the method which I now describe, and which I have commercially worked out with success, I am able to advantageously make use of the basic open-hearth furnace for low carbon high chromium steels, without any undue loss

of chromium, any more than that which occurs when producing the same grade of steel in the basic electric arc furnace, since the reduction of the chromite by ferro-silicon is carried on below the surface of the slag in intimate contact with the surface of the molten metal. A preferred procedure is as follows:

Chrome ore or chromite and ferro-silicon are first preferably ground to about 60 mesh and employed in the correct proportion to effect the reduction of the oxides of the chromium and iron, according to the following chemical reactions:



Sesqui oxide of chromium + silicon = chromium + 15 silica



Ferrous oxide + silicon = iron + silica

A slight excess of the chromite may be used to prevent any silicon from remaining unoxidized and alloying with the reduced metal. To these ingredients, slaked lime (calcium hydrate CaH<sub>2</sub>O<sub>2</sub>) is added, preferably in powdered form in sufficient quantity to combine with and partly flux the silica formed by the above reactions and to bind these ingredients together, or this bond may be provided for by using a chloride solution of an alkaline earth, such as chloride of magnesium.

They are then thoroughly mixed together, after which just sufficient water is added to make a plastic mass suitable for molding, being preferably well pugged in any suitable mill. The pugged mass is then preferably molded into relatively heavy blocks or pieces of convenient form, size and shape for the furnace men to handle, and may consist of blocks 8" x 10" x 6" weighing forty to fifty pounds. When the molded pieces or blocks are introduced on to the surface of the metal bath, being of greater density and/or weight than the slag on the bath, they will displace the slag and come into direct contact with the surface of the molten metal beneath the slag layer.

While I prefer to use ferro-silicon because of its low cost and availability, other metal silicides may be used if desired.

The molded pieces are first allowed to dry at room temperature for about 24 hours, or this drying process may be expedited by means of a current of air, and they are then, for open hearth use, preferably treated by spraying or otherwise to a milk of lime wash. After that when sufficiently dried, they are preferably transferred to any suitable drying oven or kiln, where the excess or free water is expelled. They can then be either heated up in this chamber, or transferred to a separate heating chamber which is brought up to a temperature preferably in excess of 1650° F., or in the range of temperatures between 700° C. to 1000° C., as heretofore explained. Practical operations have shown that this heating is necessary to drive off combined or colloidal water formed by the chemical reaction upon air drying of the pugged mass of ore and lime, thus not only to completely dehydrate the pieces or blocks, but also, of essential importance, to also completely degasify the same and thereby prevent the bath of molten metal absorbing gases with the danger of such bath being ruined thereby. The heated molded pieces may now be withdrawn from the heating chamber as required, and while hot are ready to be charged directly into the melting

furnace holding the bath of metal for alloying therewith.

The usual procedure may be followed in preparing the bath of molten metal in an open-hearth furnace, and the oxidizing slag formed during the melting stage is removed, after which a fresh slag of fluorspar, lime, and ferro-silicon may be added. The additions of the alloying metal are then made by introducing the molded pieces or blocks onto the metal bath, as stated.

The usual necessity of superheating the bath of metal before each addition is avoided, because the chemical reactions taking place on the surface of the metal bath produced and between the chromite and ferro-silicon are exothermic, and the heat thus given off is transferred to the metal bath and keeps the same hot and fluid. At the end of the alloying period, the bath of metal is sufficiently hot and "killed" to tap and teem into molds, where the metal rests perfectly tranquil or quiescent. The term "killed" as applied to steel means steel which is sufficiently de-oxidized to be quiescent in the molds.

An important advantage of the molded pieces or blocks is that they harden upon being kept and do not spall or disintegrate when thrown on to the metal bath at the temperature of the steel melting furnace. Also, no matter how the alloying pieces or blocks are thrown into the molten bath they will always right themselves so that the largest or heaviest side will float downwardly in direct contact with the surface of the metal bath. Due to the density and weight of the compact material of the relatively heavy molded pieces being greater than that of the molten slag, they will quickly penetrate or displace the slag and come in direct contact with the surface of the metal bath.

With the molded pieces in direct contact with the surface of the metal bath, and the intimate contact between the chromite and the ferro-silicon molded together in the molded pieces, the reduction proceeds rapidly below the slag in contact with the surface of the bath of metal and as the alloying metals are released by the reactions the molded pieces gradually diminish in size and the reduced metals pass directly into the molten bath and carry the heat with them. Accordingly, an extremely high yield or recovery of the alloying metals is obtained because substantially none of the alloying metals is oxidized and passed into the slag.

The improved method as applied to the making of chromium alloy steel provides for producing steel having 12 to 14% or more of chromium with a carbon content of not more than 0.10%. Since chromite is much less expensive than low carbon ferro-chrome, and low carbon ferro-silicon can be made economically, the alloying and reducing materials employed are relatively inexpensive.

Moreover, alloy steels having a high percentage of the alloying metals with a low carbon content can be produced by the improved method with a great saving in time, cost of material and operating, and in recovery or yield.

While I have described my improved method as applied to the production of high chromium low carbon alloy steels, the method is likewise applicable to the making of similar iron and steel alloys of numerous other alloying metals, such as tungsten and vanadium.

Also, the improved method is applicable to the production of alloy steels having a higher percentage of carbon and a lower percentage of the alloying metals.

It will be seen from the foregoing that one of the distinctive features of the present invention resides in the fact that in the so-called "piece" or block of alloying material the alloying and reducing materials are held in such compact condition that each particle of these materials is in intimate relation. Thus, full use is made of the exothermic reactions during the period of reduction, that is, the heat evolved from such reactions is carried into and disseminated throughout the bath of molten metal. This insures the alloyed metal being cast in a deoxidized and homogenous condition, thus minimizing to a very great degree the losses which usually are due to surface and edge defects. At the same time the process utilizing the pieces or blocks of alloying material made in accordance with the present invention results in an alloy having an improved molecular structure that is one in which a very fine close grain prevails with a smooth surface in the finished strip free from imperfections such as irregularities and projecting pimples or bumps. These results are quite definitely obtained because of the exothermic action taking place within and between the piece or block of alloying material and the molten metal of the molten bath. Substantial heat is evolved by this action and the alloying metal is released from the piece or block into the molten metal bath, becoming diffused or in solution therewith, and at the same time carrying the greater part of the heat of the said exothermic action with it, thereby materially contributing to maintaining the heat of the finished alloy so that it can be drawn off and teemed.

It will also be understood that in carrying out the invention that the same contemplates the use of alloying metals other than chromium, and also includes and takes into consideration the fact that more than one alloying metal may be embodied in the finished piece or block of alloying material so that the term "alloy-containing ore" as used herein is employed in a generic sense.

While I have described my improved method as carried out in the open-hearth furnace, it may be carried out satisfactorily in the electric furnace or any other suitable type or kind of furnace supplying heat throughout the process, without departing from the scope of the invention as defined in the appended claims.

I claim:

1. In a method of making alloys of iron and steel, including preparing a suitable bath of ferruginous molten metal, in any suitable type or kind of furnace supplying heat throughout the process, removing the oxidizing slag accumulated during the melting stage, and covering the metal bath with a fresh slag, composed of lime and fluorspar, to which a small quantity of ferro-silicon is added, the step of introducing on to the surface of the metal bath relatively heavy molded blocks containing one or more of the oxides of the alloying materials and a noncarbonaceous reducing agent, all in a comparatively fine state of division, being cemented together with the aid of slaked lime and water, and being of such density as to penetrate the slag and come into direct contact with the surface of the molten metal of the bath, such molded blocks, after being air dried, are sprayed over with a milk of lime wash and allowed to dry, are then heated up to a temperature in excess of 1650° F. for the purpose of freeing them from any combined water formed by the chemical reaction upon air drying of the pugged mass of ore and lime.

2. In a method of making alloys of iron and

- steel, including preparing a suitable bath of ferruginous molten metal, in any suitable type or kind of furnace supplying heat throughout the process, removing the oxidizing slag accumulated 5 during the melting stage, and covering the metal bath with a fresh slag composed of lime and fluorspar, to which a small quantity of ferro-silicon is added, the step of introducing on to the surface of the molten bath relatively heavy 10 molded blocks containing one or more of the oxides of the alloying materials and a non-carbonaceous reducing agent, all in a comparatively fine state of division, being cemented together by the aid of slaked lime and water, such 15 molded blocks having been air dried, are sprayed over with a milk of lime wash and allowed to dry, and are then heated up to a temperature in excess of 1650° F. to free them of any combined water formed by the chemical reaction upon air drying 20 of the pugged mass of ore and lime, so that, when coming into contact with the surface of the molten bath of metal, there will be no absorption of gases by the molten bath of metal from the molded blocks, and the heat developed due to 25 the exothermic chemical reaction between the materials of the molded blocks is thus transferred direct to the molten bath of metal by the precipitation of the reduced alloying metal or metals.
- 30 3. The method of preparing metal alloying material consisting of forming a compacted body of intermixed particles of alloy-containing ore and reducing agent, bonding or cementing said particles together by an hydrated oxide of an alkaline earth, pre-drying said compact body or mass, surface treating said pre-dried body or mass with a milk of lime wash, drying same, and finally heating the treated body or mass to a 35 temperature causing dehydration and degassing thereof.
- 40 4. The method of making ferruginous alloys which consists in first preparing a mass of molten metal, separately forming a compacted body of intermixed particles of alloy-containing ore and of a reducing agent bonded together by the hydroxide of an alkaline earth, subsequently subjecting the said body to a temperature not less than 700° cent., causing the liberation therefrom of free, combined and colloidal water and then 45 bringing the said body, while in a heated condition, into direct contact with the molten metal.
- 50 5. The method of making ferruginous alloys which consists in first preparing a mass of molten metal, separately preparing a compacted body 55 formed of intermixed particles of alloy-containing ore and of a silicon-containing reducing agent bonded together by the hydroxide of an alkaline earth, subsequently subjecting the said body to a temperature not less than 700° cent., causing the
- liberation therefrom of free-combined and colloidal water and then bringing the said body, while in a heated condition, into contact with the molten metal.
6. The method of making ferruginous alloys 5 which consists in first preparing a mass of molten metal, separately preparing a compacted body of intermixed particles of chrome ore and of a silicon-containing reducing agent bonded together by the hydroxide of an alkaline earth, subsequently subjecting the said body to a temperature sufficiently high to cause dehydration and degassing of said body and then bringing the latter, while in a heated condition, into direct contact with the molten metal. 10
7. The method of making ferruginous alloys which consists in first preparing a mass of molten metal, separately preparing a compacted body of intermixed ground particles of chrome ore and ferro-silicon bonded together by the hydroxide of an alkaline earth and subsequently subjecting said body to a temperature sufficiently high to cause dehydration and degassing thereof and to convert the said hydroxide into the oxide of said alkaline earth preliminary to bringing the body, 15 while in a heated condition, into surface contact with the molten metal.
8. The method of making ferruginous alloys which consists in first preparing a mass of molten metal, separately preparing a compacted body of intermixed ground particles of chrome ore and ferro-silicon bonded together by the hydroxide of calcium and subsequently subjecting said body to a temperature sufficiently high to cause dehydration and degassing thereof and to convert the said hydroxide into the oxide of said calcium preliminary to bringing the body, while in a heated condition, into surface contact with the molten metal. 20
9. The method of making ferruginous alloys 30 which consists in first preparing a mass of molten metal, separately preparing a mix, with water, of particles of alloy-containing ore and of ferro-silicon, bonding said particles together by the hydroxide of an alkaline earth, and subsequently subjecting the said mix to a temperature in excess of 700° cent. preliminary to bringing the mix into contact with the molten metal. 35
10. The method of preparing metal alloying material consisting of forming a compacted body 40 of intermixed ground particles of alloy-containing ore and of a silicon-containing reducing agent, bonding said particles together by the hydroxide of an alkaline earth, pre-drying said compacted body, and subsequently heating said body to a temperature in excess of 700° cent. causing the dehydration and degassing thereof. 45

CASIMIR JAMES HEAD.